

1,365,970.

M. H. ELVIDGE.

ROOFING.

APPLICATION FILED MAY 26, 1917.

Patented Jan. 18, 1921.

Fig. 1.



Fig. 2.



Fig. 3.



Inventor:

Morris H. Elvidge,  
by *[Signature]*  
Attorney.

# UNITED STATES PATENT OFFICE.

MORRIS HARRISON ELVIDGE, OF NEW YORK, N. Y.

## ROOFING.

1,365,970.

Specification of Letters Patent. Patented Jan. 18, 1921.

Application filed May 26, 1917. Serial No. 171,139.

*To all whom it may concern:*

Be it known that I, MORRIS H. ELVIDGE, a citizen of the United States, residing at New York, in the county of New York and State of New York, have invented certain new and useful Improvements in Roofing; and I do declare the following to be a full, clear, and exact description of the invention, such as will enable others skilled in the art to which it appertains to make and use the same, reference being had to the accompanying drawings, and to the letters and figures of reference marked thereon, which form a part of this specification.

My invention relates to what is commercially known as asphalt shingles or roofing material, and more particularly to such roofing material which has a surface of granulated or crushed slate material; and it has for its objects to provide roofing shingles or roofing material of the particular kind mentioned which will possess all the beneficial effects of such character of roofing and yet will be free from the objections of lacking uniformity of color, plain or variegated. In the manufacture of shingles or roofing material of the character mentioned the felted fabric constituting the base is saturated or impregnated with asphaltum for waterproofing purposes, and the surface to the fabric is covered or has worked into it a coating or covering of granulated or crushed slate for fire-resisting purposes and for protecting and increasing the life or durability of the roofing. While roofing shingles or material having a surface of granulated or crushed slate possess advantages over a roofing not provided with such a surface coating or covering, it is found in actual practice that the granulated or crushed slate covering or coating lacks uniformity in color and not infrequently presents streaks of different shades of the same color which detracts from the attractiveness of the roof. The colored slates most commonly used are green and red. Each of these slates, crushed or granulated, as a rule are not uniform in color. The green slate most often has in its natural state or formation a dark green and a lighter green or yellow with no regularity in the diffusion of the two colors or shades of color and when the slate in its crushed or granulated condition is applied to the asphaltic shingle or roofing these differences in shade or color are accentuated and as a consequence the surface has a streaky and

unattractive appearance. These differences in shades or colors are accentuated by reason of the crushed or granulated slate absorbing to a greater or less extent the oily constituents of the asphaltum with which the base or felt has been treated and thus the lack of harmony or uniformity in the surface is to that extent accentuated. The same is true of the red slate when crushed or granulated and applied to the roofing material as the slate absorbs oil from the asphaltum and the differences in the shade of red accentuated and the same unattractive appearance presented. These conditions also tend to deaden the colors and thus the roofing is lacking the life or warmth which contributes to its attractiveness.

I have found that by mixing the crushed or granulated green slate, *g*, with the crushed or granulated red slate, *r*, and working the same into the surface of the asphalted felt base *A*, these natural imperfections in the two colored slates are so disseminated or diffused that the slate coating or covering is freed from the streaky unattractive appearance and a surface produced of a substantially uniform variegated color, the green and the red standing out in contrasting relation so that an attractive mottled surface of contrasting intermingled particles is presented, the contrasting intermingled particles tending to relieve the dullness in color which exists when only one-colored slate is used, and the absorption of the oil of the asphaltum by the crushed or granulated slate is offset or counteracted by the contrasting colors of the mottled surface produced by the intermingling of the two distinctive colors of slate.

In the drawing Figure 1 is a front view of the asphalted felt base of the roofing; Fig. 2 a front view of the improved roofing; and Fig. 3 a face view of the roofing, on an enlarged scale for clearness of illustration.

In the manner hereinbefore described, I am enabled to produce a very attractive, effective, and artistic appearance to the roofing and at the same time have the roofing material possess advantages found to exist in an asphaltic felt base provided with a protecting coat of crushed or granulated slate. Various shades of a mottled crushed or granulated slate surface may be produced by mixing or intermingling a greater quantity of the darker material with the lighter, both as to the green and the red

colored slate, so that if a darker shade or color is desired a greater quantity of the darker material will be mixed with the lighter colored material, and on the other hand if a lighter colored roof is desired, a greater percentage of the lighter colored slate will be mixed with a smaller quantity of darker colored slate, and thus there may be produced a lighter or a darker colored surface as desired. In either case there is produced a mottled surface of a substantially uniform color made up of intermingled contrasting colors of crushed or granulated slate, free from the seriously objectionable feature of streaky discoloration such as has been found to exist when the crushed or granulated slate of one natural color alone is used. I have mentioned green slate and red slate as the colored slates ordinarily used but it is merely typical, and other colored slates than the two mentioned may be used in forming the coat or covering and be within the scope of the invention. The shingles or roll roofing of the type mentioned, that is an asphaltic felt with a coating of crushed slate, is formed in the ordinary way but the contrasting colored

crushed slate coat is formed in the manner I have described and for the purposes stated.

30

Having described my invention and set forth its merits, what I claim is:

1. The within described slate roofing comprising a base and a coating formed of a uniform mixture of crushed or granulated slates of distinctively different colors intermingled to produce a slate surface of contrasting intermingled colors of substantially uniform character throughout the coating.

2. The within described slate roofing comprising an asphalted felt base and a surface coat formed of a uniform mixture of crushed or granulated slates of distinctively different colors intermingled to produce a contrasting effect of intermingled colors of substantially uniform character throughout the coating.

40

In testimony whereof I affix my signature in presence of two witnesses.

MORRIS HARRISON ELVIDGE.

Witnesses:

E. E. HAINES,  
H. J. TAYLOR.